

(No Model.)

G. HILL.

DRAWING ROLLER FOR SPINNING AND DRAWING FRAMES.

No. 270,432.

Patented Jan. 9, 1883.

Fig. 1.



Fig. 2.



Fig. 3.



WITNESSES:

*Chas. Noga.*  
*C. Sedgwick*

INVENTOR:

*G. Hill*  
BY *Munn & G.*  
ATTORNEYS.

# UNITED STATES PATENT OFFICE.

GEORGE HILL, OF NEW YORK, N. Y.

## DRAWING-ROLLER FOR SPINNING AND DRAWING FRAMES.

SPECIFICATION forming part of Letters Patent No. 270,432, dated January 9, 1883.

Application filed June 8, 1882. (No model.)

*To all whom it may concern:*

Be it known that I, GEORGE HILL, of the city, county, and State of New York, have invented a new and Improved Drawing-Roller for Spinning and Drawing Frames, of which the following is a full, clear, and exact description.

The invention consists in a roller having a center and a covering thereof, formed of a mass of glue, oil, and leather, as hereinafter described.

Figure 1 is an end elevation of my improved roller for spinning and drawing frames. Fig. 2 is a cross sectional elevation of the same on the line  $\alpha x$ . Fig. 1. Fig. 3 is a cross-sectional elevation of a modification of the same.

I make the roller of shreds of leather of all kinds. These shreds of leather are mixed with glue and oil in the following proportions: 20 glue, (liquid,) four ounces; oil, four ounces; leather-shreds, one pound. The glue, oil, and the leather are thoroughly mixed, and are then placed in molds and pressed into the desired shape, and the leather mass A is then turned 25 off, finished, and polished. Preferably the leather mass A is molded and pressed around

a center, B, of metal, which has its periphery grooved to receive part of the leather mass to hold it on the center; or the center can be provided with a series of studs, a, projecting from the periphery into the leather mass surrounding it. These rollers can be made of different sizes, as may be required.

I am aware that it is not new to mix leather-shavings with gums and mold them into blocks 35 or cylinders or rollers; or to mix leather-shavings with hair and a compound of caseine, gluten, oxide of lead, turpentine, and gutta-percha; or to mix gum and caoutchouc with metallic layers, textile fabrics, or leather and cement; also, to cover a roll on the outside with an outer covering of leather, parchment, or paper; but

What I do not claim as new is—

A roller having a center, B, and a covering thereof, formed of a mass of glue, oil, and leather-shreds, as described.

GEORGE HILL.

Witnesses:

JAMES PETTITT,  
JOHN HIGGINS.